

## 1

3,519,626

### AMINO - METHYLOLATED MELAMINES AND PROCESSES FOR FINISHING CELLULOSE TEXTILE

Michael Thomas Beachem, Somerset, and Frederic Houghton Megson, Martinsville, N.J., assignors to American Cyanamid Company, Stamford, Conn., a corporation of Maine

No Drawing. Filed Mar. 13, 1967, Ser. No. 622,415  
Int. Cl. C07d 55/22

U.S. Cl. 260—249.6

6 Claims

#### ABSTRACT OF THE DISCLOSURE

This invention relates to new amino-methyolated melamines and to their use on cellulosic textile materials that have been dyed with direct dyes. The new amino-methyolated melamines impart crease-resistance to such materials and dyed materials so finished have improved light-fastness.

This invention relates to new compounds and to textile finishes for dyed cellulosic textile materials. More particularly, it relates to new amino-melamine-formaldehyde precondensates and their use on cellulosic textile materials dyed with direct dyes. Still more particularly, it relates to the use of new amino-methyolated melamines of the Formula I:



wherein "alkyl" is a lower-alkyl group (1-4 C atoms) and each of R and R' is hydrogen, alkyl or up to 18 C atoms, phenyl or phenyl-(lower-alkyl), any of the phenyl or said R groups, especially when R is aryl, having up to two inert radicals, such as lower-alkyl and lower-alkoxy.

The use of aminoplast resins to impart crease-resistance to cellulosics is well-known. These resin perform their function economically and efficiently without adversely affecting many of the other desirable properties of cellulosics, such as for example, fabric hand, soil resistance or fabric durability. However, aminoplast resins do, in some cases, have an adverse effect on color stability of dyed cellulosics. Thus, it is well-known that aminoplast crease-preventing finishes can cause accelerated fading of many direct dyes, i.e., the lightfastness of cellulosic textile material dyed with direct dyes is often reduced when the dyed material is after-treated with an aminoplast resin or reactant, such as a urea formaldehyde or a melamine-formaldehyde condensate. Commercial resins which have been shown to cause fading of certain direct dyes include hexa(methoxymethyl)melamine, polymethyloxolurea with slight degree of methylation, blends of partially methylated hexamethyolmelamine and urea-formaldehyde reaction products, and methylated trimethylolmelamine.

In view of the widespread use of both direct dyes and aminoplast resins on cellulosics, it is extremely undesirable to have the use of the resin for its purpose, restrict the functioning of the dye for its purpose. It is therefore

## 2

an object of the present invention to provide a means of treating direct dyed cellulosics with aminoplast resins whereby crease-resistance is imparted to the cellulosic with no substantial reduction in lightfastness other than normally encountered. It is a further object to provide cellulosics which have been direct dyed and have improved lightfastness while also exhibiting good crease-resistance by virtue of treatment with a particular aminoplast resin textile improving agent. Other objects will be apparent from the ensuing description of this invention.

It has now been discovered in accordance with this invention that methyolated melamines of Formula I impart crease-resistant properties to cellulosic textile materials without adversely affecting the lightfastness of such material dyed with direct dyes. This is a surprising discovery since cellulosics dyed with direct dyes are normally adversely affected as to lightfastness when after-treated with aminoplast textile finishes.

The textile finishing aminoplast resins used in this invention are applied to direct-dyed cellulosic textile materials by standard procedures, as by dipping, padding, spraying, etc., and the finishes are converted to an insoluble state by heating the treated fabrics in the presence of a catalyst. The dyed materials thus treated exhibit crease-resistant and wrinkle-recovery properties, and a lightfastness equal to, or even better than the untreated, dyed material.

The compounds of Formula I can be made by reacting an N-halomethylmelamine of Formula II with a compound of Formula III as follows:



wherein X is chlorine or bromine and "alkyl" and R and R' are as defined above for Formula I. The compounds of Formula II and a process for their manufacture are disclosed and claimed in U.S. Pat. No. 3,317,529, issued May 2, 1967 to Beachem et al.

Representative N-halomethylmelamines of Formula II which can be used in this invention include N-chloromethyl - N,N',N',N'',N'' - pentakis(methoxymethyl)-2,4,6-triamino-s-triazine, N - bromomethyl - N,N',N',N'',N'' - pentakis(methoxymethyl) - 2,4,6 - triamino - s - triazine, N - bromomethyl - N,N',N'',N'' - pentakis(ethoxymethyl)-2,4,6-triamino-s-triazine, N-chloromethyl-N,N',N'',N'' - pentakis(butoxymethyl)-2,4,6-triamino-s-triazine, etc.

Representative compounds of Formula III include diphenylamine, di - p - tolylamine, di-m-tolylamine, bis-(p-ethylphenyl)amine, p-methyldiphenylamine, and bis-(p-methoxybiphenyl)amine.

The reaction of compounds of Formula II with compounds of Formula III is carried out with or without a solvent, although it is preferable to use a solvent, particularly when both reactants are solids. It is also advantageous to use an acid acceptor such as an alkali metal carbonate or bicarbonate to take up the hydrogen halide which is formed by the reaction. The reaction is conveniently carried out at room temperature, although any temperature between the freezing and boiling points of

the reaction mixture may be used. Equimolar amounts of reactants can be advantageously used although an excess of either can be present without adverse effect.

The cellulosic textile materials include fibers, threads, yarns, knitted and woven cloth as well as non-woven fabrics and felted materials. These cellulosic materials will normally contain at least 50% cellulosic fibers, such as cotton, viscose, cuprammonium rayons, linen, hemp, jute, and ramie, either alone or mixed with themselves or other fibers.

The cellulosic textile materials will be dyed with the class of azo dyes known as direct dyes and so classified in the Color Index, second edition. Such dyes are characterized as anionic dyes having affinity for cellulosic fibers when applied from an aqueous dyebath containing an electrolyte. They are mainly azo dyes containing sulfonic acid groups as the sodium salts. Representative direct dyes are Direct Yellow 6 (C.I. 4001), Direct Yellow 11 (C.I. 40000), Direct Orange 26 (C.I. 29150), Direct Red 1 (C.I. 22310), Direct Red 31 (C.I. 29100), Direct Blue 2 (C.I. 22590) and Direct Green 1 (30280).

The dyed materials are treated with the textile finishes of this invention using aqueous or organic solvent solutions or dispersions which can be applied by spraying, dipping or padding according to well-known procedures. Between 0.5% and 40% solutions or dispersions are normally used. The amount of finish on the textile material can be varied, usually between 0.5% and 40% based on the weight of the textile material, with amounts between 2.5% and 15% preferably being used for practical crease-resistant and wrinkle-recovery properties. The treated fabrics are dried and then heated, preferably in the presence of a catalyst, to effect insolubility of the precondensate on the fabric (cross-linking, etc.). Curing temperatures between 275° and 400° F. for periods of about 20 minutes to 30 seconds are normally used. Suitable catalysts include those normally used for melamine-formaldehyde condensates and their etherates. These include the metal salts such as magnesium chloride, zinc nitrate and zinc chloride, ammonium salts such as ammonium sulfate, ammonium chloride, and organic amine hydrochlorides. In the case of magnesium chloride, the amount is between about 4.5% and 24%, preferably between 9% and 15%, of the anhydrous salt based on the weight of the precondensate.

The treated dyed fabric obtained by this invention will be found to have good wrinkle recovery and crease resistance normally required for commercial cellulosics. In addition, advantageously, they will be found to possess lightfastness not previously attained with aminoplast resin-treated direct-dyed cellulosics.

The following examples are presented to further illustrate this invention.

#### EXAMPLE 1



To a solution of 25.4 parts (0.15 mole) of diphenylamine in 80 parts of acetone containing 82.9 parts (0.60 mole) of potassium carbonate there is added a solution of 138.4 parts (0.30 mole) of N-chloromethyl-N,N',N'',N''-pentakis(methoxymethyl)-2,4,6-triamino-s-triazine in 80 parts of acetone. After a reaction period of about 15 hours, the reaction mixture is filtered, and the acetone is removed by distillation. A solution of the residue in benzene is washed with water. The benzene is removed by distillation and the residue is extracted with ether. The residue from the evaporation of the ether, a viscous liquid, is N - (diphenylaminomethyl) - N,N',N'',N'' - pentakis(methoxymethyl)-2,4,6-triamino-s-triazine.

#### EXAMPLE 2



To a solution of 0.15 mole of di(p-tolyl)amine in 80 parts of acetone containing 82.9 parts (0.60 mole) of potassium carbonate there is added a solution of 138.4 parts (0.30 mole) of N-chloromethyl-N,N',N'',N''-pentakis(methoxymethyl)-2,4,6-triamino-s-triazine in 80 parts of acetone. After a reaction period of about 15 hours, the reaction mixture is filtered, and the acetone is removed by distillation. A solution of the residue in benzene is washed with water. The benzene is removed by distillation and the residue is extracted with ether. The residue from the evaporation of the ether, a viscous liquid, is N - (di-p-tolylaminomethyl)-N,N',N'',N'' - pentakis(methoxymethyl)-2,4,6-triamino-s-triazine.

#### EXAMPLE 3



To a solution of 25.4 parts (0.15 mole) of diphenylamine in 80 parts of acetone containing 82.9 parts (0.60 mole) of potassium carbonate there is added a solution of 0.30 mole of N-chloromethyl-N,N',N'',N''-pentakis(ethoxymethyl)-2,4,6-triamino-s-triazine in 80 parts of acetone. After a reaction period of about 15 hours, the reaction mixture is filtered, and the acetone is removed by distillation. A solution of the residue in benzene is washed with water. The benzene is removed by distillation and the residue is extracted with ether. The residue from the evaporation of the ether, a viscous liquid, is N - (diphenylaminomethyl) - N,N',N'',N'' - pentakis(ethoxymethyl)-2,4,6-triamino-s-triazine.

#### EXAMPLE 4



To a solution of 0.15 mole of di(biphenyl)amine in 80 parts of acetone containing 82.9 parts (0.60 mole) of potassium carbonate there is added a solution of 138.4 parts (0.30 mole) of N-chloromethyl-N,N',N'',N''-pentakis(methoxymethyl)-2,4,6-triamino-s-triazine in 80 parts of acetone. After a reaction period of about 15 hours, the reaction mixture is filtered, and the acetone is removed by distillation. A solution of the residue in benzene is washed with water. The benzene is removed by distillation and the residue is extracted with ether. The residue from the evaporation of the ether, a viscous liquid, is N - [di(biphenyl)aminomethyl] - N,N',N'',N'' - pentakis(methoxymethyl)-2,4,6-triamino-s-triazine.

#### EXAMPLE 5



To a solution of 0.15 mole of di(p-ethylphenyl)amine in 80 parts of acetone containing 82.9 parts (0.60 mole) of potassium carbonate there is added a solution of 138.4 parts (0.30 mole) of N-chloromethyl-N,N',N'',N''-pentakis(methoxymethyl)-2,4,6-triamino-s-triazine in 80

parts of acetone. After a reaction period of about 15 hours, the reaction mixture is filtered, and the acetone is removed by distillation. A solution of the residue in benzene is washed with water. The benzene is removed by distillation and the residue is extracted with ether. The residue from the evaporation of the ether, a viscous liquid, is N - [di(p-ethylphenyl)aminomethyl]-N,N',N',N'',N''-pentakis(methoxymethyl)-2,4,6-triamino-s-triazine.

## EXAMPLE 6

Pad baths are prepared containing 6.25% precondensate solids and 12% magnesium chloride based on the precondensate solids in the bath.

## Pad bath A

N - (diphenylaminomethyl) - N,N',N',N'',N''-pentakis(methoxymethyl)-2,4,6-triamino-s-triazine in acetone.

## Pad bath B

N,N,N',N'',N'' - hexakis(methoxymethyl)-2,4,6-triamino-s-triazine in water.

The pad baths are applied to a sample of 80 x 80 cotton percale dyed with Direct Red 81 (C.I. 28160) at 5% O.W.F. of precondensate solids by standard padding procedure using 80% wet pickup. The treated fabrics are dried for 2 minutes at 225° F., and the finishes are cured by heating the fabrics at 350° F. for 1.5 minutes. Also, a sample of the dyed, but untreated, fabric is rinsed in water and dried. A portion of each of the fabrics of each color is washed in a home-style washing machine at 110-115° F. with water containing 0.25% of a commercial anionic surface active agent and 0.25% of sodium carbonate. The washed fabrics are dried.

Samples of the treated fabrics, both washed and unwashed, are exposed in a Fade-Ometer for 60 hours. The degree of fading of the exposed samples of fabric is measured as follows:

Spectrophotometric curves of the unexposed portion of dyed fabric and the exposed portion of dyed fabric are recorded for 21 wavelengths over the complete visual range. The spectrophotometric data are converted to colorimetric data by means of a digital computer. Numerical expressions of color in terms of 3-dimensional color coordinates are thus obtained. The two sets of colorimetric data, i.e., one set for unexposed fabric and one set for the exposed fabric, are then converted into a single color difference (in NBS units) by the system of Wyszecki, J. Opt. Soc. Am., 53, 1318 (1963). The evaluation of the colorimetric data can be done by computer.

The single number color difference thus obtained can be considered in this instance to be strength ratio figures between exposed and unexposed fabric, negative numbers indicating loss in strength, i.e. fading. The larger the color difference number, the greater the difference in the visual appearance between the two samples.

It is generally accepted that a color difference of 0.2 NBS unit is the minimum detectable amount which an experienced person can detect between two samples. The color difference for an acceptable commercial match is probably between 1.0 and 2.0 NBS units as discussed in the monograph by Judd, "Color in Business, Science and Industry," Wiley, New York, 1952.

The results of the fading measurements are shown in Table I, finishes A and B, corresponding to pad baths A and B, respectively.

TABLE I.—FADING IN NBS UNITS

|           | Initial | Washed |
|-----------|---------|--------|
| Finish A  | -7.1    | -12.2  |
| Finish B  | -12.6   | -16.7  |
| Untreated | -10.3   | -11.3  |

It can be seen that finish A is superior to finish B in resistance to light-fading and is generally equivalent to the untreated dyed fabric.

What is claimed is:

1. A compound of the formula:



wherein "alkyl" is an alkyl radical of 1-4 C atoms and R and R' are individually either hydrogen, alkyl of up to 18 C atoms, phenyl or (lower-alkoxy)phenyl.

15 2. The compound according to claim 1 which has the formula:



25 3. The compound according to claim 1 which has the formula:



30 4. The compound according to claim 1 which has the formula:



45 5. The compound according to claim 1 which has the formula:



50 6. The compound according to claim 1 which has the formula:



## References Cited

## UNITED STATES PATENTS

- 2,709,693 5/1955 Widmer ----- 260—249.6 XR  
 2,861,054 11/1958 Rust et al. ----- 260—249.6 XR  
 3,422,020 1/1969 Schmadel et al. 260—249.6 XR

## OTHER REFERENCES

Campbell et al., J. Org. Chem., vol. 26, pp. 2786-9 (1961).

70 JOHN D. RANDOLPH, Primary Examiner  
 J. M. FORD, Assistant Examiner

U.S. Cl. X.R.